

1

2,972,178

## FIBERS, YARNS AND FILAMENTS OF WATER-INSOLUBLE DEXTRAN

Malvern J. Hiler, Dayton, Ohio, assignor to The Commonwealth Engineering Company of Ohio, Dayton, Ohio, a corporation of Ohio

No Drawing. Filed Aug. 30, 1955, Ser. No. 531,587

5 Claims. (Cl. 28—82)

This invention relates to shaped articles including fibers, yarns and films consisting essentially of water-insoluble dextran.

The object of the invention is to provide new shaped articles of water-insoluble dextran, particularly fibers and films.

The dextrans are high molecular weight polysaccharides made up of anhydroglucopyranosidic units joined by molecular structural repeating 1,6 and non-1,6 linkages, at least 50% and usually a preponderant proportion of the linkages being of the 1,6 type.

The dextrans may be obtained by the action of specific microorganisms such as those of the *Leuconostoc mesenteroides* or *L. dextranicum* types on sucrose. The procedure is to inoculate a suitable aqueous sucrose-bearing nutrient medium with a culture of the microorganism or with the enzyme filtered from the culture, and incubate the mass until the dextran is produced in maximum yield, when it is separated from the fermentate and purified. The "native" dextran thus obtained normally has a high molecular weight calculated to be in the millions.

This invention contemplates the formation of fibers and films especially from dextrans which are inherently insoluble in water but soluble in aqueous alkali or from xanthates of those dextrans from which the dextran is regenerated during shaping thereof.

Microorganisms (or their enzymes) which may be used to effect biosynthesis of the water-insoluble, alkali-soluble dextran include those bearing the following NRRL (Northern Regional Research Laboratory) designations: *Leuconostoc mesenteroides* B-523, B-1118, B-1120, B-1139 and B-1144. The dextran may be the native unhydrolyzed dextran or it may be hydrolyzed to a dextran of lower molecular weight between that of the native product and that at which the hydrolyzate remains insoluble in water. The molecular weight may be as low as 50,000 depending on the ratio of 1,6 to non-1,6 linkages of the dextran.

The spinning or casting dope is obtained by dissolving the dextran or xanthate thereof in aqueous alkali, such as and preferably a 4% to 10% aqueous sodium hydroxide solution, and spinning or casting the dope through a spinneret or film-forming device into a bath in which the dextran is coagulated in the fiber or film form. Solutions of, for example, 10 to 50% of the dextran or dextran xanthate in aqueous sodium hydroxide may be used.

When the dope is an aqueous alkaline solution of water-insoluble dextran, the setting bath may be water. Dilution of the aqueous alkali extruded with the dope by the water effects coagulation of the water-insoluble dextran in the filament or film form. The bath is circulated continuously and restored to essentially neutral condition by the addition of acid so that the alkali content thereof does not reach the concentration at which the dextran is soluble.

Fibers and films formed in the water bath are with-

2

drawn from the bath, preferably stretched between godets or other suitable take-up devices or stretching means, and dried. During the stretching, the fibers or film may be subjected to a spray of warm or even hot water which maintains the article in plastic condition whereby the stretching and orientation for improvement in tenacity is facilitated.

Conventional apparatus is used.

Dextran xanthate for use in preparing the spinning dope may be obtained by mixing liquid or gaseous carbon disulfide with an aqueous slurry of the alkali derivative or the dextran (obtained by reacting the dextran with a strong alkali metal hydroxide and notably with sodium hydroxide) and maintaining the mix at a temperature of 15° C. to 25° C. until the desired degree of substitution with respect to xanthate groups is obtained, usually 2 to 4 hours using a molar ratio of alkali dextran to carbon disulfide of 1:3 to 12:1. The ester may contain an average of 0.2 to 3.0 xanthate groups per anhydroglucopyranosidic unit of the dextran.

The dextran xanthate spinning or casting dope is prepared by dissolving the xanthate in aqueous alkaline solution, e.g., 4—10% aqueous sodium hydroxide, and is spun or cast into an acid coagulating and regenerating bath, such as an aqueous solution of sulfuric acid which may contain sodium sulfate and zinc sulfate, in which bath the de-xanthation is at least initiated, with coagulation of the dextran in the fiber or film form. Baths containing 5—12% sulfuric acid, 6—20% sodium sulfate and 0.5—1.5% of zinc sulfate may be used.

The fibers or film are withdrawn from the bath, washed free of occluded bath constituents, and, preferably before or during drying, stretched between godets or the like. Softening agents, anti-blocking agents and the like may be incorporated in the films, as a step in their manufacture, if desired.

When the dope is extruded through a spinneret, the filaments may be gathered into a tow or filamentary bundle, after-processed, and the filaments of the bundle cut or otherwise disrupted to staple or discontinuous fiber.

The following examples are illustrative of specific embodiments of the invention, it being understood that these examples are not limitative.

*Example I*

A 10% solution of purified native (unhydrolyzed) *L.m.* B-523 dextran in particulate condition is dissolved in 6% aqueous sodium hydroxide at room temperature, with stirring.

The homogeneous dope thus obtained is extruded through a spinneret into continuously circulating water maintained at 50° C. The filaments formed by dilution of the aqueous alkaline solution extruded with the dextran are drawn through the bath a distance of 6 inches, withdrawn over a godet to a second godet rotating at higher peripheral speed whereby the fibers are stretched. The extent of stretching may be up to 50% of the initial length and may be facilitated by passing the fibers through a warm water bath (50° C.—60° C.) supported between the godets or by subjecting the fibers between the godets to a spray of the warm water. After drying, the fibers are collected on a spool, bobbin or other appropriate take-up device, with or without prior application of a soft finish. The fibers may be given a finishing coating of a dextran, particularly a dextran of relatively low molecular weight (5000—50,000) dissolved in water, as a substitute for starch, and dried before or during winding up thereof. These fibers have tensile strengths and elongations comparable to those of regenerated cellulose from cotton linter pulp and are useful for all textile purposes, including blending of the staple fibers.

with short fibers of other types for the production of spun yarn and so-called non-woven fabrics.

*Example II*

Example I is repeated, except that the dope comprising the aqueous alkaline solution of the water-insoluble dextran is cast through a film-forming device into the warm, circulating water, and the film is drawn through the bath for a distance of 10 inches, withdrawn, stretched while passing through water (50° C.) containing 3% of glycerol, and dried.

*Example III*

A spinning dope is prepared by dissolving 10% of native *L.m.* B-523 dextran xanthate containing an average of 2.0 xanthate groups per AGU in 6% aqueous sodium hydroxide. The dope is extruded through a spinneret into a coagulating and regenerating bath comprising an aqueous solution of 8% sulfuric acid, 11.5% sodium sulfate and 1% zinc sulfate maintained at 50-55° C., and circulated for refreshing as required. The filaments are drawn through the bath a distance of 8 inches, withdrawn, and either as a running length or after collection in an annular package or cake in a centrifugal spinning bucket are finally washed with warm water to remove occluded bath constituents, and dried. The washing and/or drying may be performed while the filaments are under stretching tension.

*Example IV*

Example III is repeated except that the dope is cast into the acid regenerating and coagulating bath through a film-forming device, the film is drawn through the bath a distance of 8 inches, withdrawn, washed and dried, and at some stage, or at all stages, between withdrawal from the bath and final drying, is subjected to tension whereby it is stretched 25% of its initial length and 5% of its initial width.

The film may be provided with a moisture-proofing coating. Particularly suitable coatings are lacquers comprising benzyl dextran or nitrodextran, the latter being a new substance which may be prepared by the method described in the pending application of L. J. Novak et al., filed February 11, 1954, Serial No. 409,781, and now abandoned.

As described in said pending application, dextran nitrate may be obtained by reacting on dextran, in solid particulate condition or dispersed in water, with concentrated nitric acid, fuming nitric acid or a mixture of nitric acid and nitrogen pentoxide, and precipitating the nitrate from the reaction mass, for instance, by means of isopropanol.

A suitable lacquer coating composition may be obtained by dissolving—

|                                | percent<br>by weight |
|--------------------------------|----------------------|
| Nitrodextran or benzyl dextran | 57.0                 |
| Dewaxed damar                  | 13.0                 |
| Dibutyl phthalate              | 23.0                 |
| Paraffin wax                   | 4.0                  |
| Zinc stearate                  | 1.0                  |

in an appropriate solvent or mixture of solvents, such as a mixture of 55.1% ethyl acetate, 3.5% denatured ethanol, and 41.4% toluene.

Nitrocellulose lacquers may also be used.

*Example V*

Example I is repeated except that the dextran dissolved in the aqueous alkali is hydrolyzed *L.m.* B-523 dextran having a molecular weight of about 50,000.

*Example VI*

Example II is repeated except that the dope extruded to form the film is a solution of hydrolyzed *L.m.* B-523

dextran of molecular weight about 200,000, in 5% aqueous sodium hydroxide.

*Example VII*

5 Example I is repeated, using a dope which is a solution of native, unhydrolyzed *L.m.* B-1118 dextran in 7% aqueous sodium hydroxide.

*Example VIII*

10 Example III is repeated except that the dope extruded through the spinneret into the acid bath is a solution of native *L.m.* B-1118 dextran xanthate containing an average of 2.3 xanthate groups per AGU in 6% aqueous sodium hydroxide.

*Example IX*

15 Example VIII is repeated except that the dope is cast into the acid regenerating and coagulating bath through a film-forming device. The film is drawn through the bath a distance of 10 inches, withdrawn, washed and dried under the tension such that it is stretched 20% of its initial length and 8% of its initial width.

*Example X*

20 Example I is repeated, using a 6% aqueous sodium hydroxide solution of native, unhydrolyzed *L.m.* B-1144 dextran.

*Example XI*

25 Example II is repeated, using as dope a 4% aqueous sodium hydroxide solution of hydrolyzed *L.m.* B-1144 dextran having molecular weight about 500,000.

*Example XII*

30 Example I is repeated using a dope consisting of a 10% aqueous sodium hydroxide solution of native, unhydrolyzed *L.m.* B-1120 dextran.

35 In general, the filaments of the water-insoluble dextran may be given a stretch of about 20% to 50% in the course of their production. Films of the dextran may be stretched 20% to 30% of the initial length, 5% to 10% of the initial width. As noted above, conventional means may be employed for spinning or casting the dope to obtain the filaments or films, and for stretching the same.

The filaments of the invention may be formed into 40 45 yarns which may be twisted in the usual way, and the yarns may be fabricated by conventional textile working methods, or disrupted to obtain a mass of discontinuous fibers for the production of a spun yarn or non-woven fabric either alone or in admixture with other fibers which latter may be natural, artificial or synthetic fibers.

50 For instance, from 15% to 65% of the dextran fibers may be carded and/or combined with fibers of cotton, rayon, nylon, "Orlon," "Dacron," "Acrlon," or mixtures of such fibers and spun into a yarn. Or yarns of the dextran fibers may be twisted with yarns formed from the other fibers or mixtures thereof.

55 For the production of non-woven fabrics, blends of the discontinuous dextran fibers with fibers of the type mentioned, rayon flock, leather scrap and so on, may be assembled in the form of a mat or bat and the assembly may be treated with an extraneous binder or adhesive which bonds the fibers into an integral coherent structure. A 3% to 10% aqueous solution of inherently adhesive dextran xanthate may be used as the binder, although other binders are also satisfactory.

60 65 In forming the bat or web, the fibers of which the dextran fibers amount to 15% to 65% by weight, may be carded together to obtain a web in which the fibers are arrayed in substantially parallelized condition, or they may be suspended in a current of air and deposited from the suspension on a reticulated collecting surface with or without the aid of suction. The dextran fibers tend to become adhesive when exposed to aqueous alkali, and this latent adhesiveness may be developed to permit autogenous bonding of mixed fibers in a yarn, non-woven

fabric or web, etc., care being taken that the action of the aqueous alkali on the fibers is controlled so that the fibers are softened to the adhesive condition while, preferably, retaining the fiber form.

The fibers and yarns and structures formed therefrom are generally useful except under conditions involving exposure thereof for any appreciable time to alkaline conditions. They may be used in constructing tire cords, in conjunction with yarns of other types, and brought to adhesive condition for bonding with rubber.

Since changes and variations may be made in practicing the invention without departing from the spirit and scope thereof, it will be understood that it is not intended to limit the invention except as defined in the appended claims.

What is claimed is:

1. As an article of manufacture an attenuated water-insoluble, dry filament of dextran of molecular weight of about 200,000 and composed essentially of dextran xanthate.

2. A shaped article consisting of fibers which fibers are composed essentially of water-insoluble dextran xanthate containing an average of 0.2 to 3.0 xanthate groups per anhydroglucopyranosidic unit of the dextran, and having a molecular weight between 50,000 and 500,000.

3. Fibers and filaments consisting essentially of water-insoluble dextran consisting of unhydrolyzed *L.m.* B-523 dextran.

4. Yarns comprising fibers consisting essentially of water-insoluble dextran xanthate containing an average of 0.2 to 3.0 xanthate groups per anhydroglucopyranosidic unit of the dextran.

5. A water-insoluble filament consisting of dextran xanthate having a molecular weight between 50,000 and 500,000 and extruded from a solution composed essentially of dextran xanthate dissolved in aqueous sodium hydroxide.

References Cited in the file of this patent

UNITED STATES PATENTS

|    |           |                |               |
|----|-----------|----------------|---------------|
| 15 | 1,559,176 | Newkirk        | Oct. 27, 1925 |
|    | 2,203,705 | Stahly et al.  | Jan. 11, 1940 |
|    | 2,394,957 | White          | Feb. 12, 1946 |
|    | 2,674,517 | Deniston       | Apr. 6, 1954  |
| 20 | 2,702,231 | Deniston       | Feb. 15, 1955 |
|    | 2,716,049 | Latour         | Aug. 23, 1955 |
|    | 2,736,652 | Novak          | Feb. 28, 1956 |
|    | 2,775,507 | Downing et al. | Dec. 25, 1956 |
|    | 2,789,915 | Bishop         | Apr. 23, 1957 |
| 25 | 2,914,414 | Novak et al.   | Nov. 24, 1959 |